

# UNITED STATES PATENT OFFICE.

DEMITY MINDELEFF, OF SAN FRANCISCO, CALIFORNIA.

## EXPLOSIVE COMPOUND.

SPECIFICATION forming part of Letters Patent No. 437,499, dated September 30, 1890.

Application filed June 11, 1890. Serial No. 355,062. (No specimens.)

*To all whom it may concern:*

Be it known that I, DEMITY MINDELEFF, of San Francisco, in the county of San Francisco and State of California, have invented 5 certain new and useful Improvements in Explosive Compounds; and I do hereby declare that the following is a full, clear, and exact description thereof.

My present invention is an improvement in 10 explosives; and its object is to produce a high-power explosive which will be largely insensitive to concussion; and it consists, essentially, in combining with nitro-glycerine alcohols, preferably methyl alcohol, which insensitizes the nitro-glycerine, and pyroxylene, as 15 will be hereinafter explained and claimed.

In preparing this explosive I take from twenty to twenty-five per cent. of nitro-glycerine and seventy-five to eighty per cent. of 20 methyl alcohol and mix the same, and then to about each one hundred cubic centimeters of the latter mixture I add from seven to ten grams of soluble pyroxylene and agitate the mass until all the pyroxylene is dissolved, keeping 25 the mixture at a temperature of from about 30° to 40° centigrade—not exceeding 40° centigrade. The resultant product will have a jelly-like appearance and consistency, and to this product I add gradually, during continuous 30 agitation thereof, nitro-glycerine in such quantities as to result in a mixture containing about seventy or seventy-five per cent. nitro-glycerine and twenty-five to thirty per cent. of methyl alcohol. This mixture is in itself a 35 powerful and insensitive explosive, and in order to increase its density I add thereto about as much soluble pyroxylene as the mixture will dissolve.

When nitro-glycerine is the second time 40 added to the solution, as above, the pyroxylene will first separate itself, but will, with time and

agitation, gradually redissolve. The final product constitutes a most powerful explosive and has a fluid or semi-fluid consistency. If it is desired to make the explosive plastic or thicken it, I add thereto powdered pyroxylene, such as is commonly known as "pressed pyroxylene."

To prevent accidents, as the above explosive is transparent and might adhere to the exterior of vessels without being noticeable, I preferably stain it with aniline, cochineal, or other pigment that would not affect its component parts. This explosive is absolutely safe. Ignited in the open air, it will 55 burn slowly until it reaches a temperature of about 280° centigrade, when it explodes. In exploding shells, cartridges, &c., the aid of both concussion and fire is employed.

Having described my invention, what I claim as new, and desire to secure by Letters Patent thereon, is—

1. An explosive compound consisting of a combination of nitro-glycerine, an alcohol, and a soluble explosive, substantially as described.

2. An explosive compound consisting of a combination of nitro-glycerine and an alcohol, and pyroxylene, substantially as described.

3. An explosive compound consisting of a combination of nitro-glycerine and methyl alcohol and pyroxylene, substantially as described.

In testimony that I claim the foregoing as my own I affix my signature in presence of two witnesses.

D. MINDELEFF.

Witnesses:

S. POSTAWKA,  
T. H. ALEXANDER.